

No Drawing.

Application filed May 5, 1915. Serial No. 25,917.

*To all whom it may concern:*

Be it known that I, OTTO I. METZGER, a citizen of the United States, residing at Far Rockaway, in the county of Queens and State 5 of New York, have invented a new and useful Composition of Matter to be Used for Jewelry, Pins, Metallic Springs, and other Metallic Articles.

My composition consists of the following 10 ingredients combined in the proportion stated, viz: copper 15 parts, silver 5 parts, zinc 10 parts. These metals are first melted and then mixed. The composition is then hardened by alternately heating and suddenly cooling. On reheating and cooling gradually, the metal becomes elastic or soft depending upon the degree of heat to which it has been subjected and to the rapidity with which it is cooled.

20 Variations in the proportions of copper and silver used, copper within the limits of from 33 $\frac{1}{3}$ % to 56 $\frac{2}{3}$ % and silver within the limits of from 10% to 33 $\frac{1}{3}$ % will show variations in the quality of the composition.

25 For example, 17 parts of copper with three

parts of silver gives the quality of toughness to the composition. As the proportion of copper is decreased and the silver correspondingly increased, the composition becomes less tough or more brittle, so that when equal parts of copper and silver are employed the composition is extremely brittle. Therefore, the proportion of parts will be varied depending upon the to which the composition is to be put. Zinc may be varied between the limits 28% and 42% of the total composition, with corresponding relative variations in the copper and silver.

I claim:

The herein described composition of matter consisting of 15 parts of copper, 5 parts of silver, and 10 parts of zinc, substantially as described.

Dated, New York, May third, 1915.

OTTO I. METZGER

Witnesses:

EDWARD A. EATON,  
RALPH M. SUTPHEN.